

## UNITED STATES PATENT OFFICE

2,263,823

METHOD OF PRODUCING AND TREATING  
ALUMINUM ALLOY CASTINGS

Walter Bonsack, South Euclid, and Walter M. Weil, Shaker Heights, Ohio, assignors to The National Smelting Company, Cleveland, Ohio, a corporation of Ohio

No Drawing. Application December 6, 1939,  
Serial No. 307,882

5 Claims. (Cl. 148—3)

This invention relates to aluminum base alloys, and more particularly to a method of heat treating aluminum base alloy castings containing one or more hardening ingredients.

It is an object of this invention to provide a method for increasing the strength and hardness of heat treatable aluminum alloy castings by heating the castings for a relatively short time.

It is another object of this invention to provide a simpler and more efficient method of heat treating aluminum alloy castings in a comparatively short time to give them considerably improved properties.

In order to improve the strength and hardness of aluminum alloy castings by heat treatment, a solid solution having a substantial amount of hardening constituents dissolved therein should be first obtained, and a substantial proportion of these dissolved hardening ingredients should be precipitated in highly dispersed form from the solid solution. In any given heat treatable alloy, the larger the amount of hardening ingredients in the solid solution the greater is the potentiality for hardening.

The solid solution may be prepared by the so-called "solution heat treatment" of the metal as described in the Bureau of Standards Bulletin No. 337, of 1919, and later in the Jeffries and Archer Patent No. 1,572,487, granted February 9, 1926. By this method the castings are heated at temperatures around 900° F. to 1000° F. for at least seven hours, and usually for a considerably longer time, to dissolve the hardening constituents.

In carrying out such solution heat treatments the time of holding the casting at the high temperature is important. A relatively long heating period is generally necessary to cause a sufficient proportion of the precipitated hardening ingredients to be dissolved to accomplish a substantial improvement in properties. Even after the solid solution has been formed in the manner above set forth, the hardening constituents will be precipitated again in substantially ineffective form if the casting be allowed to pass slowly through the temperature range where precipitation may occur relatively rapidly. It is therefore desirable, in order to obtain the benefits of solution heat treatment, that the hot casting be quenched relatively quickly to the temperature of the precipitation zone, or below, to avoid appreciable crystallization of the hardening constituents during the cooling.

A solid solution of hardening ingredients may 55

also be prepared by quenching an aluminum alloy casting as soon as practical after it has solidified in the mold, but the proportions of hardening and strengthening ingredients in the solution obtained by this method are somewhat less than those obtained by the solution treatment usually employed, so that the potentiality for hardening and strengthening by utilizing one of the well-known aging processes is considerably less. This method has not, therefore, displaced the solution treatment in the preparation of those castings where the most improved properties, such as strength, ductility and hardness, are desired.

When a casting is removed from the mold relatively quickly after it is solidified and quenched, not all of the hardening constituents are precipitated from the solid solution. It has been found that such a casting, however, even though quenched from the mold may be heated from room temperature through a temperature range where precipitation of the hardening constituents usually occurs, up to the ordinary solution heat treating temperatures, without precipitating a substantial amount of dissolved hardening ingredients. If this is done, one may heat the quenched casting at a solution heat treatment temperature, which may be considered as a temperature where solubilization of hardening ingredients of the alloys occurs, for a comparatively short time to produce results equal or superior to those obtained by the longer solution heat treatment.

In accordance with our invention, heat treatable aluminum alloy castings of superior strength and hardness are obtained by quenching the castings after solidification in the mold, and while they are hot enough to have a substantial quantity of the hardening ingredients in solid solution, heating the quenched castings at solution heat treatment temperatures for a comparatively short time, again quenching the castings and giving them a suitable aging treatment.

This invention applies to articles cast from aluminum alloys containing hardening constituents, whether such articles be cast in sand or metal molds. The articles are preferably removed from the mold and quenched as soon as is practical after solidification of the metal takes place, so as to retain larger amounts of hardening constituents in solid solution. Even when the castings have cooled below the ordinary solution heat treating temperatures before they are quenched, sufficient of the ingredients are retained in solid solution to substantially shorten the time of heating subsequently required. It is

preferred, however, that the castings be removed from the molds and quenched at a temperature above 850° F. or 900° F., depending on the composition of the alloy.

The quenched castings which have a substantial quantity of dissolved hardening constituents should preferably be heated as rapidly as possible through the precipitation temperature range to the solution heat treating temperature. They may be heated in any suitable heat treating furnace. When heated in a gaseous atmosphere, the furnace should preferably be of such a design as to cause the heating of the casting to be relatively rapid.

The solution temperatures vary of course with the alloy used, but may generally be considered as temperatures which are slightly below the melting point of the eutectic, and for most aluminum alloys are usually in the range of 850° F. to 1050° F. The preferred solution temperature for any heat treatable aluminum alloy is 10° to 20° below the melting point of the eutectic.

For example, the aluminum-silicon alloys are treated at temperatures between 950° F. and 1050° F., whereas the aluminum-copper alloys are treated at lower temperatures, between 900° F. and 1000° F., and aluminum-zinc alloys are heated to temperatures still lower, such as 850° F. to 950° F. When the previously quenched casting is heated a relatively short time in the temperature range appropriate to the alloy, a solution of the hardening ingredients is obtained which is equal to or superior to that obtained by the relatively long conventional heat treatments heretofore used.

In practicing the invention, an hour or less is usually sufficient at a solubilizing temperature, and only seldom is it desirable to heat the alloy at such temperature for as long as about 2 or 3 hours. It will, therefore, be seen that a tremendous saving in cost of heat treating is made by the application of this invention. Thus, it has been found that castings quenched from the mold and heated for only about an hour at a suitable temperature for the alloy and then again quenched, have even greater potentiality for hardening and strengthening when suitably aged than the usual castings which have been heated 8 or 10 hours at 950° F. and quenched.

Although with castings previously quenched from the mold a heating period of 15 minutes or so at the solution or solubilizing temperature produces marked improvements, it is preferred that the heating be continued for a longer time, such as about an hour or two, to obtain a more uniform product having a larger percentage of hardening constituents in solid solution. The time to produce a desired solid solution of hardening ingredients is of course dependent on the temperature, and the higher the temperature or with a given alloy the nearer the temperature used is to the melting point of the eutectic of the alloy, the shorter will be the time required. It has been found that castings having excellent properties may be obtained by holding them at a suitable solubilizing temperature for about a half hour or so, quenching and aging.

The quenching may be in any medium which cools the casting sufficiently rapidly to retain the hardening constituents in solid solution. However, as a general rule, when cooling or quenching of the casting from the solution heat treating temperature is relatively rapid, a greater potential improvement of the hardness and strength of the metal of the casting may be ob-

tained. The casting may be quenched to room temperature, or to the temperature at which it is desired to age the casting, thus avoiding the re-heating of it to the aging temperature. In order to develop the inherent physical properties of the casting, a suitable aging treatment is usually given castings after quenching.

If the alloy used is one which readily increases in hardness at room temperature, the treated casting may be aged at room temperature. It is, however, often desirable or necessary that the aging be carried on at elevated temperatures, such as that of boiling water or temperatures up to about 450° F., to improve the characteristics of the castings.

The aging time and aging temperatures generally used for solution heated alloy castings are applicable to the castings heat treated in accordance with this invention. The aging time depends upon the particular alloy being aged and the properties of the metal desired. For any given properties, the required aging time will depend upon the temperature, and with a higher temperature a shorter aging time may usually be used. It is rarely necessary to age more than fifteen hours, and for many castings the time may be considerably less.

The method set forth above is applicable to heat treatable aluminum alloys, such as those having one or more of the usual commercial alloying constituents, as copper, zinc, magnesium, silicon, manganese and nickel.

The following example illustrates the invention:

35 A molten aluminum alloy containing 4% copper, 2% silicon, 1% iron and 0.5% zinc was poured into a permanent mold at operating temperature. The test bars were quenched in water from the mold at a temperature between solidification temperature and mold temperature. The quenched castings were transferred to a heat treating furnace, heated for 1½ hours or so at about 950° F., again quenched in hot water and aged 2 hours at 212° F. When tested, the hardness of the casting was 65 Brinell, the tensile strength 40,000 lbs./sq. in., and elongation 7.5%.

When the same alloy was cast in the same manner and in the same mold but slowly cooled to room temperature, it had to be heated for about 7 hours at about 950° F. to get about 37,000 lbs./sq. in. tensile strength a hardness of 60 Brinell, and elongation of 7%.

Furthermore, it is to be understood that the particular compounds disclosed and the procedure set forth are presented for purposes of explanation and illustration, and that various equivalents can be used and modifications of said procedure can be made without departing from our invention as defined in the appended claims.

60 What we claim is:

1. The process of producing an aluminum alloy casting, which comprises pouring the molten metal in a gravity permanent mold, removing the casting from the mold promptly after solidification, and before it has cooled below about 850° F., quenching it while it is hot enough to have a substantial quantity of hardening ingredients in solid solution, heating the quenched casting to a temperature at which solubilization of the hardening ingredients occurs, holding the casting at such temperature for fifteen minutes to three hours, and again quenching the casting from a solubilizing temperature.

75 2. In a process for producing castings from

aluminum alloys containing copper, the steps which comprise quenching the casting from the mold relatively quickly after it has solidified and before it has cooled below about 850° F., so that an effective proportion of the hardening ingredients is still in solid solution, heating the quenched casting to a temperature to cause solubilization of hardening ingredients not in solution, maintaining the casting at such solubilizing temperature for less than three hours, again quenching the casting from a solubilizing temperature to a suitable aging temperature, and aging the casting.

3. The process of producing an aluminum alloy casting, which comprises pouring the molten metal into a gravity mold, removing the casting from the mold promptly after solidification, quenching before it has cooled below about 850° F., heating the quenched casting between about 850° F. and the melting point of the lowest melting eutectic in the alloy, maintaining this temperature for from fifteen minutes to one hour, again quenching the casting from a temperature above about 850° F., and artificially aging the

casting above room temperature and below about 450° F. to improve its properties.

4. The process of producing an aluminum alloy casting, which comprises pouring the molten metal in a mold, removing the casting from the mold before it has cooled to 850° F. and quenching it, heating the quenched casting at temperatures between 850° F. and 1050° F. for fifteen minutes to three hours to cause solubilization of the hardening ingredients, and again quenching the casting.

5. The process of producing an aluminum alloy casting, which comprises pouring the molten metal into a gravity mold, quenching the casting from the mold before it has cooled below about 850° F., so that a substantial quantity of hardening ingredients is in solid solution, heating the quenched casting at a temperature at which solubilization of the hardening constituents of the alloy occurs, and quenching the casting from a solubilizing temperature.

WALTER BONSACK.  
WALTER M. WEIL.